

## UNITED STATES PATENT OFFICE.

PAUL RABE, HERMANN STÖTTER, AND BERTHOLD WENK, OF LEVERKUSEN-ON-THE-RHINE, AND WILHELM SCHEPSS, OF WIESDORF-ON-THE-RHINE, GERMANY, AS-SIGNORS TO GRASSELLI DYESTUFF CORPORATION, OF NEW YORK, N. Y., A CORPORATION OF DELAWARE.

## PROCESS OF PRODUCING DYEINGS FAST TO LIGHT.

No Drawing. Application filed December 15, 1926, Serial No. 155,101, and in Germany December 22, 1925.

This invention relates to a process for making dyeings of acid and basic dyestuffs on fibers which are fast to light.

We have found that this can be accomplished by precipitating complex compounds of tungstic acids or molybdic acids or tungstic-molybdic acids or mixtures thereof and especially the phospho-tungstic acids, the phospho-molybdic acids, and the phospho-tungstic-molybdic acids upon the fiber by means of organic fixators preliminary to the dyeing thereof with acid or basic dyestuffs.

By organic fixators we mean organic materials such as aliphatic and aromatic amines and their derivatives, phenols and their derivatives, thio-compounds and compounds having an alcoholic residue. The use of tannin as an organic fixator is excluded.

The so treated fibers are now able to take up acid and basic dyestuffs giving dyeing having a particularly enhanced fastness to light as compared with similar dyeings made by using tannin in place of the organic fixators referred to.

We have found, further, that the light-fastness property of dyeings of acid and basic dyestuffs may be enhanced by treating the said complex compounds precipitated on the fiber with reducing agents, for example, the commonly used bisulfites, hydrosulfites, formaldehyde or the like.

In this case it is possible also to omit the treatment of the fibers with the so-called organic fixators since the treatment of complex tungstic acid and molybdic acid compounds upon the fiber with the said reducing agents effects the fixation thereof.

After-treatment of mordanted dyeings obtained according to this process with salts or acids, in the well known manner, for example, with copper acetate, phospho-tungstic-molybdic acid, or the like, may be resorted to, effecting an enhanced fastness to washing.

## Example 1.

Cotton is treated with a 1% solution of benzidine hydrochloride, squeezed out, and treated with a 1% solution of phospho-tungstic-molybdic acid at 70° C. The well-rinsed cot-

ton is then dyed, in the customary manner, with the dyestuff obtainable from tetramethyldiaminobenzhydrol and dibenzylaniline-disulfo acid. There is obtained thereby a clear violet dyeing, distinguished from the basic violet dyeings on tannin-mordanted cotton by a remarkable fastness to light.

Instead of the phospho-tungstic-molybdic acid above-mentioned, there may be used phospho-tungstic acid or phospho-molybdic acid.

## Example 2.

Cotton is treated as described in Example 1 above, substituting phenol in place of the benzidine hydrochloride as the fixator. There is obtained, by dyeing the fiber so treated with the dyestuff obtainable from ethyl-benzyl-m-toluidine sulfo acid and p-diethylaminobenzaldehyde, a blue dyeing that is characterized by an outstanding fastness to light as contrasted with the basic blues obtainable on tannin-mordanted cotton.

Analogous results are obtained by substituting, for phenol itself, 1,8-dihydroxynaphthalene-3,6-disulfo acid or other phenols such as thio-phenol.

## Example 3.

Cotton is treated as described in the preceding examples, with the substitution of tetramethyldiaminobenzhydrolsulfo acid (Ber. 27, 1405) as fixator. The treated cotton is dyed with the dyestuff disclosed in German patent No. 287,003, yielding a greenish blue dyeing of great fastness to light.

## Example 4.

Acetate silk is treated with dibenzylaniline-m-sulfoacid as fixator. Dyeing with the dyestuffs obtainable from tetramethyldiaminobenzhydrol and ethylbenzyl-m-toluidine sulfo acid yields a dyeing of an intense violet shade possessing great fastness to light.

## Example 5.

Cotton is treated as hereinbefore described with the exception that, in place of the previously mentioned fixators there is sub-

stituted grape sugar. Upon dyeing with the dyestuff mentioned in Example 2, a light blue dyeing is obtained which is characterized by a great fastness to light as contrasted to 5 analogous dyeings on tannin-mordanted cotton. In place of grape sugar may be used dextrine, starch, cane sugar, milk sugar or the like. With similar results one may use cyclo-  
10 hexanol and the like.  
10 The washing-fastness of the dyeings obtained according to Examples 1-5 may be still further improved by after-treatment with salts or acids in the known manner, for example, with copper acetate, phospho-tung-  
15 stic-molybdic acid or the like.

*Example 6.*

The fiber, treated as described in Example 5, is dyed with China green (Schulz-Julius, 20 1914, 495), yielding a clear green dyeing of great fastness to light.

*Example 7.*

Cotton is padded with a 1% solution of 25 phospho-tungstic-molybdic acid, squeezed out, and treated with a solution of sodium bisulfite and sulfuric acid; rinsed, and, in the ordinary manner, dyed with 1% China green crystals or other basic dyestuff.

30 We claim:

1. In the process of dyeing fiber the step which comprises precipitating on the fiber by means of an organic fixator a complex acid containing at least one metal of the 35 group including molybdenum and tungsten.

2. In the process of dyeing fiber the step which comprises precipitating on the fiber by means of an organic fixator a complex phosphoric acid containing at least one metal 40 of the group including molybdenum and tungsten.

3. In the process of dyeing fiber the step which comprises precipitating on the fiber by means of an organic fixator a complex phosphoric acid containing tungsten.

4. In the process of dyeing fiber the step which comprises precipitating on the fiber by means of an organic fixator a complex phospho-tungstic-molybdic acid.

5. The process of dyeing fiber which comprises precipitating on the fiber by means of an organic fixator a complex acid containing at least one metal of the group including molybdenum and tungsten and then dyeing 55 the fiber by means of a dyestuff of the group including the acid and basic dyestuffs.

6. The process of dyeing fiber which comprises precipitating on the fiber by means of an organic fixator a complex phosphoric acid containing at least one metal of the group including molybdenum and tungsten and then dyeing the fiber by means of a dyestuff 60 of the group including the acid and basic dyestuffs.

7. The process of dyeing fiber which com-

prises precipitating on the fiber by means of an organic fixator a complex phosphoric acid containing tungsten and then dyeing the fiber by means of a dyestuff of the group including the acid and basic dyestuffs.

8. The process of dyeing fiber which comprises precipitating on the fiber by means of an organic fixator a complex phospho-tungstic-molybdic acid and then dyeing the fiber by means of a dyestuff of the group includ- 70 ing the acid and basic dyestuffs.

9. The process of dyeing which comprises precipitating on the fiber by means of an organic fixator a complex acid containing at least one metal of the group including molybdenum and tungsten, treating the precipitated compound on the fiber with a reducing agent and dyeing the fiber by means of a dyestuff of the group including the acid and basic dyestuffs.

10. The process of dyeing which comprises precipitating on the fiber by means of an organic fixator a complex phosphoric acid containing at least one metal of the group including molybdenum and tungsten, treat- 90 ing the precipitated compound on the fiber with a reducing agent and dyeing the fiber by means of a dyestuff of the group including the acid and basic dyestuffs.

11. The process of dyeing which comprises precipitating on the fiber by means of an organic fixator a complex phosphoric acid containing tungsten, treating the precipitated compound on the fiber with a reducing agent and dyeing the fiber by means of a dyestuff of the group including the acid and basic dyestuffs.

12. The process of dyeing which comprises precipitating on the fiber by means of an organic fixator a complex phospho-tungstic molybdic acid, treating the precipitated compound on the fiber with a reducing agent and dyeing the fiber by means of a dyestuff of the group including the acid and basic dyestuffs.

13. The process of dyeing fiber which comprises precipitating on the fiber by means of an aromatic phenolic compound containing not more than three phenolic OH groups, a complex phosphoric acid containing at least one metal of the group including molybdenum and tungsten, and then dyeing the fiber by means of a dyestuff of the group includ- 110 ing the acid and basic dyestuffs.

14. The process of dyeing fiber which comprises precipitating on the fiber by means of an aromatic phenolic compound containing not more than three phenolic OH groups, a complex phospho-tungstic-molybdic acid, and then dyeing the fiber by means of a dyestuff of the group including the acid and basic dyestuffs.

15. The process of dyeing fiber which comprises precipitating on the fiber by means of phenol a complex phosphoric acid contain- 125

ing at least one metal of the group including molybdenum and tungsten, and then dyeing the fiber by means of a dyestuff of the group including the acid and basic dyestuffs.

5 16. The process of dyeing fiber which comprises precipitating on the fiber by means of phenol a complex phospho-tungstic-molybdic acid, and then dyeing the fiber by means of

a dyestuff of the group including the acid and basic dyestuffs. <sup>10</sup>

In testimony whereof, we affix our signatures.

PAUL RABE.  
HERMANN STÖTTER.  
BERTHOLD WENK.  
WILHELM SCHEPSS.